

# UNITED STATES PATENT OFFICE.

ROBERT ABBOTT HADFIELD, OF WESTMINSTER, ENGLAND.

## MANUFACTURE OF METAL ROLLS.

1,318,748.

Specification of Letters Patent. Patented Oct. 14, 1919.

No Drawing.

Application filed June 24, 1919. Serial No. 306,448.

To all whom it may concern:

Be it known that I, Sir ROBERT ABBOTT HADFIELD, baronet, F. R. S., a subject of the King of Great Britain and Ireland, residing at Westminster, England, have invented Improvements in or Relating to the Manufacture of Metal Rolls, of which the following is a specification.

Considerable difficulty has heretofore 10 been experienced in producing rolls of a durable character suitable for rolling metals or alloys, particularly metals or alloys of a hard nature. The present invention has reference to improvements in the manufacture of rolls of the kind referred to designed 15 to overcome the difficulty referred to.

For this purpose, a roll according thereto is made of high quality steel such as nickel-chromium steel, or chromium steel, or nickel 20 steel, forged or cast approximately to shape, then annealed and machined to the required finished shape, after which it is heat treated in such a manner, as by heating it to a hardening temperature and quenching it in a 25 suitable cooling liquid, that the enlarged or working portion of the roll is rendered hard, tough and durable.

The carbon in the nickel chromium steel, used may advantageously be of the order of 30 about .6%, the nickel of the order of from about 2 up to say 3½% and the chromium of the order of from about 2 to 3%. In the case where the rolls are made of chromium steel, or nickel steel, the chromium or nickel 35 may vary up to 4 or 5%. The invention however is not limited to the particular percentages of the elements mentioned. Usually the steel will be free from or low in manganese. Satisfactory results have been 40 obtained by forging down an alloy steel blank containing about .67% of carbon, about 2% of nickel and about 2% of chromium, to approximately the shape and dimensions of the required roll, then annealing the roll, as 45 for instance by heating it to from 700 to 800° C., say to about 765° C., and allowing it to cool slowly, as for instance in the furnace in which the heating was effected, then machining the annealed roll to the desired 50 finished shape, and heating the enlarged or working portion thereof uniformly to a hardening temperature of say about 875° to 880° C., the journals or trunnions being heated to a less temperature, and then 55 quenching the roll in oil. Thus treated, the said enlarged portion of the roll had a hard-

ness corresponding to from about 93 to 98 as determined by the schleroscope. The journals of the roll will usually be of a less degree of hardness than the central or working portion thereof. The degrees of hardness mentioned are only given by way of example. The hardness can be varied to suit the particular use to which the roll is to be applied. The hardening temperature may in 65 some cases be taken up to say 950° C.

In some cases it may be found advantageous to temper the hardness of the roll to a suitable extent. This can be done in any known or suitable way. For example, it 70 can be done by heating the roll, after quenching it for a greater or less time in a suitable cooling medium, to a temperature say for example up to about 300° C. and then immersing it in a suitable cooling medium, for example oil at ordinary temperature, or it may be cooled in air.

Also, the hardened steel roll, whether tempered or not, may be heated uniformly 80 to a temperature that may vary from 50° C. up to 250 or 300° C., preferably from 100° to 200° C., by immersing it in a bath of oil heated to the desired temperature, allowing it to remain in the oil until it attains the 85 temperature thereof, then withdrawing it from the oil, and allowing it to cool slowly in air or otherwise. In this way the toughness of the hardened, or hardened and tempered, steel roll can be increased in an 90 advantageous manner without reducing or unduly reducing its hardness.

The heating of the roll to the desired hardening temperature may conveniently be effected in a gas burning furnace, the heat 95 being directed mainly on to the central portion of the roll that is to be rendered hard and tough. Usually the roll will be heated while supported in a vertical position and its lower journal or lower and upper journals may be protected to some extent against overheating by placing it or them in or covering them with protecting means, during some portion of the heating process. The roll may conveniently be rotated to insure uniform heating thereof and the heating 100 be effected slowly and, it may be, in stages, so as to gradually heat the roll to the desired hardening temperature. The surface of the roll may, if desired, be suitably protected 105 against oxidation during the heating.

The quenching of the roll may also be done 110 by suspending it vertically and dipping it

endwise into a bath of oil or other suitable quenching medium.

When the roll is cast, instead of forged, approximately to shape, it may, especially in the case of high nickel steels, be annealed by heating it to a much higher temperature than that hereinbefore mentioned, say for example up to a temperature of about 1,200 or 1,300° C.

10 After the hardening process, or hardening and tempering or toughening processes, the roll can be suitably finished, as by grinding and polishing in known ways, to finally adapt it for any particular use.

15 Instead of forging or casting the roll initially, approximately to shape, it may be machined approximately to shape, from a suitable ingot or blank.

Instead of making the whole roll of nickel 20 chromium steel, or chromium steel, or nickel steel, as described, it may be composed of an inner portion or core of iron or steel of a different and, it may be, cheaper quality than nickel chromium steel or chromium 25 steel, or nickel steel, and an outer tubular portion or covering of nickel chromium steel or chromium steel or nickel steel, heat treated as described to render it hard, tough and durable, the two portions being rigidly 30 secured together in any convenient way, the outer portion being that portion actually used in rolling. In either case the roll may be made hollow if desired.

Rolls constructed as described may be of 35 plain cylindrical or other desired shape and are specially adapted to the cold rolling of metals and metallic alloys.

What I claim is:—

1. In the manufacture of a metal roll, 40 forming the metal roll of nickel chromium steel in which the carbon present is of the order of about six tenths per cent., the nickel of the order of from about two to three and one half per cent. and the 45 chromium of the order of from about two to three per cent., heating the working portion of said roll to a high temperature and hardening it while at the desired hardening temperature by a suitable cooling medium, tempering the hardened portion of the roll and 50 afterward toughening the hardened and tempered portion of the roll by heating it to a temperature not exceeding about 300° C. and allowing it to cool.

55 2. A process for the manufacture of a roll of the kind herein referred to, said process consisting in forming the roll approximately to shape of nickel chromium steel, annealing said roll by heating it to a high temperature 60 and allowing it to cool slowly, finishing said roll to shape, supporting it in a heating space and heating its enlarged working portion to a high temperature, hardening said portion of the roll while it is at the desired 65 hardening temperature by immersing the

heated roll in oil, and tempering said hardened working portion of the roll by heating it to a temperature of about 300° C. and then cooling it.

3. A process for the manufacture of a roll 70 of the kind herein referred to, said process consisting in forming the roll approximately to shape of nickel chromium steel, annealing said roll by heating it to a high temperature and allowing it to cool slowly, finishing said 75 roll to shape, supporting it in a heating space and heating its enlarged working portion to a high temperature, hardening said portion of the roll while it is at the desired hardening temperature by immersing the 80 heated roll in oil, tempering said hardened working portion of the roll by heating it to a lower temperature than the hardening temperature and cooling it and toughening the hardened and tempered portion of the 85 roll by heating it uniformly in oil at a temperature not exceeding about 300° C. and afterward allowing it to cool slowly.

4. A process for the manufacture of a metal roll, said process consisting in heating 90 the enlarged working portion of a roll, formed of high quality steel, to a high temperature, hardening said portion of the roll by cooling it while at the desired hardening temperature by a cooling medium, tempering 95 the hardened portion of the roll by heating it to a lower temperature than the hardening temperature and cooling it and toughening the hardened and tempered portion of the roll by heating it uniformly in oil to a temperature of from about 50 to 300° C. and allowing it to cool.

5. A process for the manufacture of a metal roll, said process consisting in heating 100 the enlarged working portion of a roll 105 formed of high quality alloy steel and of the required shape to a high temperature, in a heating space by the action thereon of flame while it is being rotated, hardening said portion of the roll while at the desired 110 hardening temperature by quenching it in a cooling medium, tempering the hardened enlarged working portion of the roll by heating it to a suitable tempering temperature and cooling it and afterward toughening 115 the hardened and tempered portion of the roll by heating the roll in a bath of oil uniformly to a temperature of from about 50° C. to about 300° C. and allowing it to cool slowly.

6. A process for the manufacture of a roll 120 of the kind herein referred to, said process consisting in forming said roll approximately to shape, and of nickel chromium steel of approximately the composition 125 herein set forth, annealing it, then forming it to the required finished shape, suspending it with its axis vertical in a heating space, heating its enlarged working portion uniformly to a high temperature by the direct 130

application thereto of heat while slowly rotating it, quenching the heated roll, at the desired hardening temperature in a cooling liquid to harden its enlarged portion, tempering the hardened enlarged portion of the roll, and toughening the hardened and tempered portion of the roll by immersing the roll in a bath of oil heated to a temperature not exceeding about 300° C., and

10 allowing it to cool slowly.

7. A process for the manufacture of a metal roll of the kind herein referred to, said process consisting in forming a roll of nickel chromium steel containing about six

15 tenths to seven tenths per cent. of carbon, about two to three decimal five per cent. of nickel, and about two to three per cent. of chromium, annealing said roll, forming it

to the required finished shape, suspending it with its axis vertical in a heating space, 20 heating its enlarged working portion to a high temperature, quenching it while at a hardening temperature of from about 875 up to about 950° C., by immersing it in a cooling liquid, tempering the hardened enlarged portion of the roll as set forth, and afterward toughening the hardened and tempered enlarged portion of the roll by immersing the roll in a bath of oil heated to a temperature of from about 100 to 200° C., 30 removing it from said bath after it has been uniformly heated to this temperature and allowing it to cool slowly.

Signed at 22 Carlton House Terrace, London, England, this fourth day of June, 1919. 35

ROBERT ABBOTT HADFIELD.